

Nov. 18, 1941.

R. E. WAGNER

2,262,785

METHOD OF AND APPARATUS FOR TREATING GREENSAND

Filed June 8, 1937

2 Sheets-Sheet 1



INVENTOR.  
RICHARD E. WAGNER

BY

Emery, Varney, Whitemore & Co.  
ATTORNEYS.

Nov. 18, 1941.

R. E. WAGNER

2,262,785

METHOD OF AND APPARATUS FOR TREATING GREENSAND

Filed June 8, 1937

2 Sheets-Sheet 2



Fig. 3.



Fig. 5.



Fig. 2.



Fig. 4.

INVENTOR.

RICHARD E. WAGNER

BY

Emery, Varney, Whitemore & Dix  
ATTORNEYS.

## UNITED STATES PATENT OFFICE

2,262,785

METHOD OF AND APPARATUS FOR  
TREATING GREENSAND

Richard E. Wagner, Forest Hills, N. Y.

Application June 8, 1937, Serial No. 147,035

3 Claims. (Cl. 23—111)

This invention relates to method of and apparatus for treating greensand or glauconite to improve its water softening properties and to the improved product, and has for an object the provision of improvements in this art.

The invention relates particularly to an improved heat treating process for greensand or glauconite.

It has been proposed to heat greensand to improve its qualities as a softener. If the heating is conducted with free exposure to air the greensand will disintegrate, so it has also been proposed to heat the greensand in a reducing atmosphere. In most cases warning has been given that the temperature must not exceed 600° C. or the greensand will be spoiled. In some instances a maximum temperature of 650° C. has been permitted if a reducing atmosphere is maintained. The suggestion made was to heat the greensand in the presence of heating flames. Practically, it is difficult to obtain efficient heating up to 650° C. with a reducing flame; so it seems safe to assume that some heating at the beginning with an oxidizing flame was required. Moreover, in order to obtain the required temperature with a reducing flame and with the usual type of kiln or oven it is necessary to apply heat for a long time, making the process undesirably slow.

Then too, in order to obtain the most immediate effects of the flame it is brought into direct contact with the greensand. This is objectionable because if even a small portion of the flame is oxidizing it may injure some of the material or reduce its efficiency and structural strength as far as water softening purposes are concerned. It also leaves carbon in the greensand.

In some previous processes the greensand has been mixed with oil or other reducing agents in the attempt to avoid oxidizing conditions or to create a reducing atmosphere, but it is obvious that the higher temperatures are hard to thus obtain and that the introduction of a foreign substance into the greensand may be objectionable for many reasons.

Again, the greensand has been treated in batches, a given quantity being heat treated for a considerable time and then replaced by another batch. This is very objectionable because it is difficult to heat a large volume of material throughout, and moreover, the quality of different batches is likely to vary greatly.

According to the present invention the greensand is heated to a higher degree and under entirely new conditions from what has ever before been proposed for producing a base exchange

material, so far as is known. This heat treatment is conducted under carefully controlled conditions to insure that the greensand will not be injured. This results in a product which is distinctly superior to any similar product which has heretofore been produced.

A feature of the invention is the heating of the greensand by the indirect application of heat when the heating means involves oxidation as does a fuel flame. It is thus possible to use an oxidizing flame and obtain efficient combustion and a temperature as high as may be desired without injuring the greensand in any manner.

Where electrical heat is cheap it may be used in place of fuel combustion heat and since electrical heat is non-contaminating and in some cases reducing, there is no objection to placing the heating means in the same chamber with the greensand to be heated. But in any case atmospheric air and oxidizing conditions are substantially excluded.

Another feature of the invention is the application of heat to a thin body of material whereby every particle may be quickly and uniformly heated. This has many advantages over heating large bodies of material.

Another feature of the invention is the provision of a continuous operation. Since the material is heated in a thin body it may be passed along and heated in a continuous stream. This makes for greater uniformity in the product and very materially speeds up production.

Another feature of this invention is the method and means to heat the greensand rapidly and almost instantaneously to a high temperature and cool quickly in an oxygen-free atmosphere.

Another feature of this invention is the method and means to heat the greensand rapidly and almost instantaneously to a high temperature and to cool quickly in a reducing atmosphere.

Another feature of this invention is the method and means to heat the greensand to a high temperature and maintain a non-oxidizing or reducing atmosphere without adding reducing agents.

Another feature of this invention is the method and means to heat greensand to a high temperature and maintain a non-oxidizing or reducing atmosphere due to the natural agents present in the greensand itself.

Another feature of the invention is the method and means for protecting the highly heated greensand by the vapor of occluded or combined water driven off from the greensand.

Another feature of the invention is the method

and means for protecting the highly heated green-sand by the vapor of sulphur or its compounds driven off or formed by heating the greensand.

Another feature of the invention is the method and means for agitating and fully exposing green-sand particles while heating them to rapidly and uniformly harden each grain; also to accomplish this in a continuous manner and fully protecting the greensand from oxidizing conditions.

Another feature of the invention is the provision of apparatus for subjecting the greensand to a high temperature under the specified environment but which will not be injured materially or destroyed under such conditions.

Another feature of the invention is the method and means for hydrating the heat-treated green-sand and the ability of the heat-treated green-sand to withstand this treatment to produce an improved final product.

Another feature of the invention is the method and means for hydrating the heat-treated greensand with an acid or an alkali or both and the ability of the heat-treated greensand to withstand this treatment to produce an improved final product.

Another feature of the invention is the improved final product and its ability to withstand regeneration with either salts or acids whereby a greater range of base-exchange reactions may be efficiently performed by the greensand.

Other objects and features will be apparent to those skilled in the art from the following description of an exemplary embodiment of the invention.

In order to illustrate the principles of the invention one specific embodiment will be described in detail, reference being made to the accompanying drawings wherein:

Fig. 1 is an elevational view of a plant embodying the invention;

Fig. 2 is a vertical section at the feeding end of the apparatus, the view being taken on the line 2—2 of Fig. 1;

Fig. 3 is a vertical section through the furnace, the view being taken on the line 3—3 of Fig. 1;

Fig. 4 is a vertical section at the discharge end of the heating drum, the view being taken on the line 4—4 of Fig. 1; and

Fig. 5 is a vertical section at the discharge end of the hydrating drum, the view being taken on the line 5—5 of Fig. 1.

In carrying out this process with the apparatus shown, greensand is preliminarily washed and classified to remove fines, clayey inclusions and coarse particles and is then dried until most of the adhering dampness is driven off. The remaining particles are composed principally of glauconite but contain some clayey matter, some iron sulphide, free silica and other substances.

The dried greensand is elevated by any suitable means and dropped into a feed hopper 10 provided with an adjustable spout 11 to deposit the greensand in a feed or pick-up trough 12. By adjusting the vertical position of the slideable spout sleeve 11a the height of the body of sand 13 in the trough 12 may be varied to vary the amount of feed as will be explained presently.

Means are provided for passing the greensand in a thin body or layer through a heating zone without coming in contact with the heating medium or harmful gases of fuel combustion and oxidizing media, to quickly heat it to any desired temperature and to cool it, before coming in

contact with air, to a point where air will have no harmful effect upon it.

The means herein shown for this purpose comprise an inclined rotary drum 16 mounted on trunnions 17 and rotated through gears 18 and 19 by a shaft 20 driven by a motor M1.

The main portion of the drum 16 is disposed within a furnace 21 heated by any suitable means such as an oil burner 22. In order to obtain 10 efficient utilization of the combustion heating gases they are required to pass around the ends of longitudinal baffles 23 extending from the sides of the furnace to the sides of the drum. The used gases pass out a stack 24. The drum is 15 heated exclusively from the outside when combustion products are used for heating so the flame may be made as oxidizing as desired to create any temperature required. None of the combustion gases come in contact with the green-sand being treated.

The portion of the drum within the furnace which is highly heated may be made of a metal which is highly resistant to heat without losing its shape or deteriorating under the conditions 20 to which it is subjected. For example a 28% chromium steel may be used. A cast special alloy steel has been found most suitable for the very high temperatures which are preferred. The portions 16a, 16b of the drum which extend outside the furnace walls may be formed of a lower quality metal. They may be joined to the central portion by flanges 16c which preferably include heat insulating material such as asbestos to reduce the heat passing from the central portion 25 to the end portions.

In order to completely exclude air from the interior of the drum both ends are closed by suitable heads. The upper head 16d may be provided with a small opening 25 to permit such 30 gases as are generated in the drum to escape. The entire upper end of the drum may be enclosed by a hood 28 evacuated through a pipe 29 by a gas pump P operated by a motor M2. The gases are discharged from the pump through 35 a discharge pipe 30.

Material is fed into the drum 16 by a curved feed pipe or scoop 31 secured to and rotating with the drum. The height of the sand in the trough 12 determines the length of arc along 50 which the feed pipe engages the sand and hence the amount of sand which is fed in at each rotation of the drum.

The greensand passes as a thin stream down the drum as it rotates due to the pitch or mechanical feeding means of the drum. During this passage the greensand is rapidly heated until near the end of the furnace for approximately two feet it is at a red or white heat, that is, at 55 700° C. or over. When a drum of chrome steel alloy is used the temperature may be much higher than 700° C. Temperatures as high as 1200° C. have been employed with a metal drum. If a refractory lined drum heated interiorly by electrical or other suitable non-contaminating means 60 were employed even higher temperatures might be attained and successfully used. The material passes through this zone quite rapidly, say in one or two minutes. The time of passage 65 through the entire heating zone or furnace is very short, say five or ten minutes. The heating 70 is thus seen to be very rapid.

The gases generated by heating the greensand 75 may include steam from the moisture and water of occlusion or composition driven off, and sul-

phur, possibly in some combined form, from the iron sulphides contained in the greensand. These gases will insure that non-oxidizing or reducing conditions will exist within the drum.

The treated greensand is rapidly cooled in the end portion 16b of the drum. If the cooling of the drum by air is not sufficiently rapid the drum may be further cooled by streams of water from a pipe 32 or otherwise. The heat-treated greensand is not exposed to the air until it has cooled sufficiently to be unharmed when so exposed.

The relatively cool greensand is discharged from the drum by a helical discharge pipe 33 secured to and rotating with the drum. The pipe 33 opens into one side of the lower end of the drum so that a quantity of greensand enters it at every turn. The successive charges of greensand form air seals in the lower loops of the coiled pipe 33 to positively exclude air from the drum.

The heat-treated greensand may be used immediately for water softening purposes but it may be preferred to hydrate it or otherwise further treat it to improve its water softening characteristics. Hydration alone might be effected simply by the use of the greensand in a water softener but it has been found that by combining other treatment with the hydration the greensand is improved and made more suitable for market. An alkali treatment or an acid treatment or both may be employed.

After the greensand has cooled sufficiently it may be transferred in any desired manner, as by conveyor, vehicle or blower to bins or other places of storage, shipment or further treatment. For further discussion, it will be assumed that it is carried to a hydration device. As shown herein, the greensand is finally discharged from the end of the pipe 33 into a hopper 34 leading into the waste gas discharge pipe 30 previously mentioned. An adjustable baffle plate 35 in the pipe causes the gases to pass without escaping to any extent and to create a suction on the injector principle to entrain the same with the gases. The time of passage from the pipe 33 to the hopper 34 is very brief and the gases in the pipe 30 are non-oxidizing in nature so the greensand is not oxidized even if fairly hot. If desired, an air excluding hood may be placed around the discharging greensand. It is to be understood that if the greensand is properly protected from air it may be transferred at a higher temperature than it would if exposed to air.

The heat-treated greensand is hydrated in any suitable manner. For example, it may be blown through the pipe 30 into a hopper 38 and thence fed into a hydrator 39.

Hydration may be effected in the hydrator by water, preferably heated, by acids such as hydrofluoric acid or phosphoric acid, by alkalis such as caustic soda, or other suitable substances. The substance selected will be the one which is most appropriate for the results to be achieved.

If hydration alone is desired, water is adequate, if iron is to be removed suitable acids may be used; if silica or aluminum or both are to be removed alkalis such as caustic soda or acids such as hydrofluoric acid may be used; and so on.

While the natural action of water in a zeolite softener would eventually hydrate the greensand and build up or increase its exchange value and efficiency without hydration before use in the softener, it is more practical to hydrate in various manners and ways to prepare this material

for its ultimate use. Then again, it is generally assumed that the exchange capacity of a zeolite to a large extent is due to its surface area; that is, by increasing the surface area the exchange capacity is increased. Because of the heat treatment employed above, it is possible with various methods to increase the surface area of the greensand. For example, by subjecting the greensand which has been treated according to the present process with caustic soda the greensand will not only become hydrated but at the same time the caustic will remove silica and alumina without weakening the grain structure, thereby increasing the surface area so that the exchange capacity of this material can be increased 100% over that of the raw greensand otherwise processed for water softening purposes. Materials produced on a commercial scale according to the present invention consistently show an increase in porosity, since the finished product—on a dry basis—weighs only 78 pounds per cubic foot against 90 pounds per cubic foot for the raw dry greensand. This increase in porosity can best be accounted for by the expanding action of the water of combination contained within the greensand molecule when subjected to a high temperature and a short heating period; while the increase in hardness of the grains is undoubtedly due to a simultaneous sintering action. The use of caustic for hydration or rehydration is well known but due to the particular pre-treatment employed herein special advantages are obtained.

In a similar manner, the greensand which has undergone the heat treating process described above can be hydrated or treated with an acid which instead of removing silica and alumina by means of caustic will remove iron and other matter soluble in acids, thereby increasing the surface area and the exchange capacity. Such acid treated material can or may be used on waters of different character and for obtaining different results. While sodium chloride is generally used for regenerating zeolites, the above-treated material can be regenerated with alkalis or acids to form alkaline or acid zeolites for various purposes.

Assuming that caustic soda is used in the hydrator, the greensand which has been heat-treated according to this process will withstand the action of a much higher concentration of caustic solution without disintegrating than will greensand made by previous processes.

The greensand from the hopper 38 is blown or otherwise conducted into the liquid bath of caustic soda or other hydrating material in the hydrator. The bath is preferably kept heated, say at about 230° F. or boiling in any suitable manner as by blowing live steam into the bath by a pipe 40. The hydrator drum is constantly rotated to keep the greensand and liquid thoroughly mixed together. The greensand may remain in the hydrator about one hour on an average. Additional caustic or caustic solution may be added as desired, while the apparatus continues in operation, through a feed device 45.

Instead of or in addition to heating the bath by steam it may be heated by an oil burner 41, the drum being suitably enclosed in furnace walls and a stack provided.

Means are provided for removing the hydrated greensand from the drum. Preferably such means are adjustable to regulate the amount of the greensand removed. As shown, the drum is provided at the outlet end with buckets 42 which

elevate the greensand and drop it into a hopper 43 leading to a chute 44. By adjusting the axial position of the hopper 43 in the drum it is made to intercept more or less of the length of the buckets 42 and hence more or less of the material discharged from the buckets.

Some liquid will be removed with the sand but this may later be washed out and the sand subsequently dried.

By operating the heat treating device to deliver a constant quantity of treated greensand of uniform quality, it is made practicable to operate the hydrator continuously.

No attempt will be made to explain the theory underlying the reactions which occur during the process. The steps of the process have been explained with sufficient particularity to enable a person skilled in the art to practice the invention. So it is believed sufficient to state that the material produced has been found superior to any other known for general water softening purposes. It is quite black in color instead of green like most greensands; and is harder and will withstand the disintegrating action in softening apparatus without breaking up or sludging better than any other known greensand, or any zeolite at all whether natural or artificial, for that matter.

While one embodiment of the invention has been described in considerable detail to furnish a clear understanding of the principles of the invention it is to be understood that the invention may be variously embodied within the lim-

its of the prior art and the scope of the subjoined claims.

I claim:

1. The process of treating greensand to improve it for base exchange reactions which comprises, subjecting the greensand in a thin body to a temperature of 950° C. or above for a short period of 5 to 10 minutes in a closed chamber in an inert or reducing environment produced from the greensand itself free from air and combustion flames and gases, and then quickly cooling the greensand free from air and combustion flames and gases.
2. The process of treating greensand to improve it for base exchange reactions which comprises, subjecting the greensand in a thin body to a temperature of 950° C. or above for a short period of 5 to 10 minutes in a closed chamber under inert or reducing conditions free from air or combustion flames and gases.
3. The process of treating greensand to improve it for base exchange reactions which comprises, passing the greensand alone in a thin stream continuously through an enclosed heating chamber to subject all particles intimately to a temperature of 950° C. or above for a short period in an inert or reducing environment produced from the greensand itself, free from air and combustion flames and gases, cooling the greensand quickly, and blowing the greensand to a hydration chamber by gases withdrawn from the heating chamber.

RICHARD E. WAGNER.